



US005565417A

# United States Patent [19]

Salvia

[11] Patent Number: 5,565,417

[45] Date of Patent: Oct. 15, 1996

[54] HYBRID SERIES TRANSITION METAL POLYMER COMPOSITE SETS

[76] Inventor: **Vincent F. Salvia**, 1533 N. Woodward Ave., Ste. 160, Bloomfield Hills, Mich. 48304

[21] Appl. No.: 494,383

[22] Filed: Jun. 26, 1995

[51] Int. Cl.<sup>6</sup> ..... C10M 125/00; C10M 147/02

[52] U.S. Cl. ..... 508/167; 508/168; 508/169; 508/181

[58] Field of Search ..... 252/25

[56] References Cited

U.S. PATENT DOCUMENTS

|           |         |                 |       |        |
|-----------|---------|-----------------|-------|--------|
| 3,437,593 | 4/1969  | Bellavin        | ..... | 252/25 |
| 3,496,003 | 2/1970  | Simon-Vermot    | ..... | 252/25 |
| 3,847,826 | 11/1974 | Ivanov          | ..... | 252/25 |
| 4,052,323 | 10/1977 | Feneberger      | ..... | 252/23 |
| 4,414,241 | 11/1983 | Quella et al.   | ..... | 252/25 |
| 4,557,839 | 12/1985 | Tubbs           | ..... | 252/23 |
| 4,626,365 | 12/1986 | Mori            | ..... | 252/25 |
| 4,715,972 | 12/1987 | Pacholke        | ..... | 252/25 |
| 4,787,993 | 11/1988 | Nagahiro        | ..... | 252/25 |
| 4,892,669 | 1/1990  | Marcora et al.  | ..... | 252/25 |
| 5,407,590 | 4/1995  | Salvia          | ..... | 252/25 |
| 5,433,870 | 7/1995  | Nakamura et al. | ..... | 252/25 |
| 5,464,586 | 11/1995 | Wagner          | ..... | 252/25 |

Primary Examiner—Ellen M. McAvoy

[57]

## ABSTRACT

The present invention provides a specific hybrid series of

transition metal polymer matrix composite sets which create durable friction reducing, wear, and corrosion resistance characteristics which can be used in a powder or liquid form, or, which can be bonded to a desired surface at ambient temperature. The specific components are combinations of polytetrafluoroethylene and molybdenum disulfide, polytetrafluoroethylene and tungsten disulfide, or tungsten disulfide and molybdenum disulfide. This invention brings together the unique properties of organic chemistry (polytetrafluoroethylene) and inorganic chemistry (tungsten disulfide, or molybdenum disulfide). This invention creates a synergistic interaction which enhances the wear resistance properties of polytetrafluoroethylene while simultaneously improving the friction reducing properties of molybdenum disulfide, or tungsten disulfide. The material functionality of this invention is greatly improved over the individual friction-reducing and wear-resistance capabilities of its constituent components being used independently. The invention comprises varying mixture sets of polytetrafluoroethylene and molybdenum disulfide, polytetrafluoroethylene and tungsten disulfide, or molybdenum disulfide and tungsten disulfide, depending upon the desired friction and wear-resistance needed. This invention can be introduced into the lubrication of mechanical components in powder form, in a colloidal dispersion, or, can be applied and caused to bond directly to a substrate surface through a variety of mechanisms and manners to form a lubricious and wear-resistant layer ranging from 0.5 microns to 60 microns thick.

26 Claims, No Drawings

## HYBRID SERIES TRANSITION METAL POLYMER COMPOSITE SETS

### FIELD OF THE INVENTION

This invention specifically relates to the unique and unanticipated improvement of lubrication and wear resistance characteristics realized through a combination of the inorganic transition metal dichalcogenides (TMD) molybdenum disulfide (MoS<sub>2</sub>) and tungsten disulfide (WS<sub>2</sub>) in separate combinations with organic polytetrafluoroethylene (PTFE). The invention identifies the unique interaction that occurs when combining PTFE, MoS<sub>2</sub> and WS<sub>2</sub>, in specific composite sets. The invention addresses three particular composite set combinations, 1) PTFE and MoS<sub>2</sub>, 2) PTFE and WS<sub>2</sub>, and 3) WS<sub>2</sub> and MoS<sub>2</sub>. In addition, this invention discusses a variety of ways in which these new compounds can be introduced to and/or applied to substrata.

### BACKGROUND OF THE INVENTION

Friction is a significant problem in all mechanical systems and can result in wear, noise, the generation of excess heat and energy consumption. The reduction of friction is an ever growing concern in manufacturing and transportation based industries because of the escalating costs of electrical power for running machinery and equipment, and fuel for internal combustion engines. Manufacturing equipment as well as engine and drive train components include a large number of moving parts. Even a small reduction in friction will have a great economic impact upon manufacturing and transportation based industries.

Petroleum based lubricants, either in a liquid or solid form, such as oils, greases are very important in reducing friction in a variety of mechanical systems. Petroleum based lubricants, relative to TMDs however, have low load carrying abilities which limits their effectiveness and their usefulness in high load bearing applications. In some instances systems include precision parts or working environments that would be contaminated by breakdown and outgassing of liquid lubricants.

Dry lubricants have been developed in response to the various shortcomings of liquid lubricants. Dry lubricants generally comprise materials which are fairly inert and which have a lamellar structure which causes them to be lubricious. Among some of the widely utilized dry lubricants are graphite, talc, molybdenum disulfide, tungsten disulfide, niobium disulfide, and boron nitride. Other dry lubricant materials such as ditellurides and diselenides of various group V and VI metals are also employed. In some instances, particles of a lubricous polymer, such as PTFE or other such fluorocarbon polymers, are utilized as dry lubricants. Dry lubricant materials are generally employed in a loose powdered form, or they may be used in combination with a liquid lubricant. Loosely applied lubricant coatings wear away and must be continually renewed. Further, loose particles of lubricant can contaminate a variety of systems.

In response to these shortcomings, various efforts have been made to develop permanent dry lubricant coatings. The term "permanent" as used to describe the lubricant is meant to define a lubricant film which is tightly bonded and integral with the workpiece surface, and is in contrast to lubricant films which are merely deposited upon the surface. In some instances, articles are coated with fluorocarbon polymers so as to provide a highly lubricous surface; however, these coatings are generally soft and have a tendency to migrate off a substrate surface when exposed to pressures.

Various processes have been developed for bonding dry lubricant coatings to the surfaces of various articles. U.S. Pat. Nos. 3,632,368 and 3,644,133 (the disclosures of which are incorporated herein by reference) describe a method for permanently bonding a coating of tungsten disulfide to metallic workpieces. The process disclosed therein uses a modified sandblasting technique wherein atomically clean surfaces are impacted at a fairly high rate of speed with particles of dry lubricant material. This application discloses an impingement bonding technique.

The present invention is directed toward producing a lubricious wear-resistant compound adapted to refrain from migrating away from highly loaded contact areas. Use of the present invention enables the production of vehicles as well as processing equipment, tools, and manufacturing equipment which are longer lasting, more energy efficient and more reliable. These and other advantages of the present invention will be readily apparent from the discussion and description which follow.

### PRIOR ART

It is known to use graphite with alkylene homopolymer or copolymer (Ref. U.S. Pat. No. 4,052,323) as a high temperature lubricant for the purpose of hot-working of metals. This art contains relatively large particle size graphite (100 to 900 microns) and uses an alkylene homopolymer which functions in a different manner from this present invention. Graphite's lubricating characteristics require interaction with water molecules versus the interaction of its internal molecular structure. It does, however, demonstrate another example of synergistic benefit gained through unique organic and inorganic compound combinations.

The development of a synergistic lubricant additive (Ref. U.S. Pat. No. 4,557,839) using molybdenum disulfide mixed with antimony thioantimonate (SbSbS<sub>4</sub>) uses smaller particles of MoS<sub>2</sub> (0.1 to about 10 microns), however, this art does not address the unique benefits derived from the composite sets of this invention (PTFE and WS<sub>2</sub>, or PTFE and MoS<sub>2</sub>, or WS<sub>2</sub> and MoS<sub>2</sub>) as discussed in this present invention.

The synergistic mixture presented in this invention has not been found in prior art.

### SUMMARY OF THE INVENTION

The present invention provides a durable, wear-resistant lubricious material which can be caused to bond to a desired surface, or dispersed in a colloidal suspension, so as to provide reduced friction, wear and energy consumption. The specific components are tungsten disulfide (WS<sub>2</sub>), molybdenum disulfide (MoS<sub>2</sub>) and, polytetrafluoroethylene (PTFE). This invention brings together the unique properties of organic chemistry (PTFE) and inorganic chemistry (MoS<sub>2</sub>, WS<sub>2</sub>) which creates a synergistic interaction optimizing the friction reducing wear resistance properties of each material. The invention consists of a composite set compound of either PTFE and WS<sub>2</sub>, PTFE and MoS<sub>2</sub>, or WS<sub>2</sub> and MoS<sub>2</sub>, which can be applied to a substrate through a variety of mechanisms and manners to form a lubricious and wear-resistant layer ranging from sub-micron layers one up to 60 microns thick.

The compound may include various mix ratios of PTFE, MoS<sub>2</sub>, or WS<sub>2</sub> depending upon the desired coefficient of friction and material load carrying characteristic properties tailored to specific applications. For example, a mixture of the composite sets would be prepared for general use—using

equal amounts of each component—or “use specific” in which the mixture is formulated to meet specific use requirements. For example, under lower load needs use a higher percentage of PTFE with MoS<sub>2</sub>, or PTFE with WS<sub>2</sub>. Where higher load needs exist, one would use a higher percentage of MoS<sub>2</sub> with PTFE, or WS<sub>2</sub> with PTFE, or for extreme loads, WS<sub>2</sub> and MoS<sub>2</sub>.

In operation, the present invention presents several methods of applying the invention as a permanent, wear-resistant, lubricous coating to a substrate which exists in either a dry or liquid environment.

#### Dry Application

The dry application of this invention requires a thorough surface cleaning to the substrate for the deposition of any of the material composite sets. After surface cleaning preparation is complete there exists a number of ways to deposit the invention.

The step of cleaning the workpiece may comprise the steps of providing a liquid based cleaning bath and immersing the workpiece in the cleaning bath. Alternatively, the step of cleaning the workpiece is abrasively cleaned. In some instances, a protective coating may need to be applied to the workpiece concomitant with the step of cleaning to insure the workpiece remains free of contaminants.

Impingement bonding this matrix composite set of PTFE and MoS<sub>2</sub>, PTFE or WS<sub>2</sub>, or WS<sub>2</sub> and MoS<sub>2</sub>, onto a workpiece allows for a deposition which does not require binders, adhesives or excessive temperatures. More specifically the method includes the steps of: 1) providing at least one workpiece, 2) cleaning the surface of the workpiece to remove substantially all contaminants therefrom, impingement bonding the invention as described onto at least a portion of the workpiece, and 3) a mechanical impingement process whereby the workpiece is placed in a rotating container which contains the formulated invention mixture. The mechanical impingement process can be enhanced through the introduction of a material carrying the compound and associated burnishing media.

The invention may be deposited in a stream of carrier gas which is directed onto the workpiece with force sufficient to cause the lubricant to bond to the surface of the workpiece. Sufficient force is provided by pressurizing the gas stream to approximately 30–200 psi. The WS<sub>2</sub> or MoS<sub>2</sub> bind with the PTFE and the new compound forms a tenacious physical bond at the molecular level when such conditions exist.

#### Liquid Application

Liquid application of the invention requires first converting the invention's composite sets from a dry powder form into a stabilized colloidal suspension. The invention is readily converted into this format using existing technology that is known to those skilled in the art of creating particle suspension in colloidal solution. Once the invention is placed in solution it may be introduced into an end product where reduced friction and wear-resistance is desirable. The invention in solution, or in dry powder form, may be added directly or, if desired, may be premixed into another carrier media such as an oil or other type of lubricant or general liquid media. In this form the invention may be added to such things as engine crank cases, manual transmissions, rear end differentials, bearing applications or any application desired. Once entered into a liquid lubricating media, a portion of the invention will transmigrate from its suspended colloidal form to become bonded to the working surface of the substrates in contact with. Once bonded it will maintain its friction and wear-resistance protection and work in conjunction with the balance of the material which remains in solution.

These and other objects and aspects of the invention will become apparent in a detailed description of the invention presented hereinafter.

#### DETAILED DESCRIPTION OF THE INVENTION

There is disclosed a transition metal polymer composite set of materials which provide a durable, wear-resistant lubricous material. The invention consists of composite sets of PTFE and MoS<sub>2</sub>; PTFE and WS<sub>2</sub>; and, WS<sub>2</sub> and MoS<sub>2</sub>. The combination of these materials within each composite set creates an unexpected result when considering the individual characteristics. Individual characteristics are as follows: Polytetrafluoroethylene (PTFE) is an organic homopolymer from tetrafluoroethylene monomer. It is a linear carbon chain encapsulated within a shroud of fluorine atoms. The alignment of the atoms is such that a balance exists between the internal electropositivity and an external electronegativity which yields no net charge difference and contributes to its inert chemical nature. With this molecular structure PTFE exhibits a low coefficient of friction resulting from the weak bond forces between the external positioned fluorine atoms and substrates in which they come in contact with. PTFE has a specific gravity of 2.13–2.22, a dynamic coefficient of friction of 0.1, and is a relatively soft material having a hardness rating of 50–65 on the Shore D scale. PTFE is available from the Du Pont Company, Little Falls Centre I, Willmington, Del. 19880-0810. Tungsten disulfide (WS<sub>2</sub>) and molybdenum disulfide (MoS<sub>2</sub>) are diatomic cross-linked molecular structures which form a lubricous layer. Both materials are naturally inert. The absolute density of tungsten disulfide (WS<sub>2</sub>) is 7.4 grams per cubic centimeter. Tungsten disulfide is commercially available from sources such as Osram Sylvania of Towanda, Pa. The molecular weight of molybdenum disulfide (MoS<sub>2</sub>) is 160.06 with a nominal density of 4.96 grams per cubic centimeter. Repurified MoS<sub>2</sub> is available from sources such as Climax Molybdenum Corporation, a division of Amex, Inc. of Greenwich, Conn. The crystal structure of both materials is that of a laminar, layer-lattice type, in which a planar layer of tungsten and molybdenum atoms are interspersed between two layers of sulfur atoms. The load carrying capabilities of these MoS<sub>2</sub> and WS<sub>2</sub> has been measured as high as 500,000 psi. Although the materials described herein have been used separately and individually as dry film lubricants and in solutions for oils and greases, there has been no invention created that addresses the unique, beneficial characteristics of the materials working in union with each other. WS<sub>2</sub> and MoS<sub>2</sub> are classified as transition metal dichalcogenides (TMD) which includes the disulfides, diselenides and ditellurides of Ti, Zr, Hf, V, Nb, Cr, Mo and W. These compounds form trigonal prisms with six chalcogen atoms to form the hexagonal type crystal. The beneficial lubricating characteristics of WS<sub>2</sub> and MoS<sub>2</sub> are related to the layered crystal structures (the large spacing and the weak Van der Waals bonding) between the sandwiched layers. Differences in lubricating behavior among the TMD compounds are attributable to the distribution of electrons on the composing atoms. In WS<sub>2</sub> and MoS<sub>2</sub>, there are six non-bonding electrons available to completely fill the band which physically confines the electrons within the crystal structure. This creates a net positive charge on the surface of the layers which promotes easy shear through electrostatic repulsion.

In PTFE, the carbon atoms are arranged in a linear manner with the fluorine atoms totally encapsulating them. As the

external charge of the PTFE molecule carries a uniform negative charge which causes low interfacial forces as a result of electrorepulsion. Hence, a lubricating effect occurs because of the ease of shearing between layers of PTFE and between the PTFE and the substrate onto which it is deposited.

This invention creates an improvement over the known benefits and unique characteristics of MoS<sub>2</sub>, WS<sub>2</sub> and PTFE, individually, while addressing a limitation in the deposition and retention of PTFE on a surface without binders, adhesives or in high temperature applications.

PTFE as a single dry film lubricant, will not adhere to a substrate and will "migrate" away from even moderately loaded contact areas and lose its effectiveness under extreme pressure working surfaces. The present invention causes the PTFE to be molecularly interlocked within the its composite companion, either MoS<sub>2</sub> or WS<sub>2</sub>, on a substrate surface at the point of contact. The PTFE and MoS<sub>2</sub>, PTFE and WS<sub>2</sub>, or WS<sub>2</sub> and MoS<sub>2</sub> materials are "interlocked" or "driven into" each other during the deposition process. This phenomenon, called intercalation, prevents migration off of the working surface area by the PTFE.

PTFE is a relatively soft material and is unsuited for many tribological applications. Converting PTFE into equivalent load carrying properties yields a maximum of only 120 psi measured at 1200 feet and a velocity of 10 feet per minute. At slightly higher ranges PTFE's load carrying properties reduce to only 2.5 psi at 1000 feet per minute for distance of 2500 feet.

WS<sub>2</sub> and MoS<sub>2</sub> are crystalline structures. When bonded onto a bearing surface these materials will still not cover the surface 100%. Resultant microscopic "pin holes" will expose enough surface so that oxidation may occur as water molecules bond to the exposed surface. The PTFE component of this invention will provide increased effectiveness during the intercalation process and reduce, and conceivably eliminate, the amount of exposed surface which will create an improved or fully corrosion resistant lubricious surface.

The use and application of WS<sub>2</sub> or MoS<sub>2</sub> provides a thin film coating, however, it is difficult to obtain a layer greater than 0.5 to 3 microns. The introduction of PTFE as a composite with MoS<sub>2</sub> or WS<sub>2</sub>, through the cross bonding affinity the material has to demonstrated, allows for a process to create a lubricious, wear resistant thin film coating of up 60 microns in a relatively short period of time—as little as 20 minutes in one mechanical application.

This invention allows the lubrication and wear resistant properties of PTFE with MoS<sub>2</sub>; PTFE with WS<sub>2</sub>; or WS<sub>2</sub> with MoS<sub>2</sub>, to be efficiently realized, providing optimal tribological properties not before experienced. It uniquely combines the beneficial characteristics which exist within the organic and inorganic materials at the molecular and atomic level to create a superior wear resistant, lubricious and corrosion resistant material. If desired, the material can be readily applied at room temperature without the use of binders or adhesives. The composite material sets adapt easily to create a colloidal solution which will allow transfer of the material to the desired substrate during the normal lubrication cycles of engine, gear, or other mechanical, manual or electronic devices.

The invention identifies that it is possible to calibrate mixture ratios of specific composite sets (PTFE and MoS<sub>2</sub>, PTFE and WS<sub>2</sub>, WS<sub>2</sub> and MoS<sub>2</sub>) to address the specific needs of each and every application. This includes the ability to build a heavier concentration of material, if required by specifications, by using an equal mix of the PTFE with

MoS<sub>2</sub>, or WS<sub>2</sub>; or to create a thinner coating as required by using a lower ratio of PTFE within the composite. The range of mix ratios of this invention for either composite of PTFE with MoS<sub>2</sub>, PTFE with WS<sub>2</sub>, or WS<sub>2</sub> with MoS<sub>2</sub>, slides along a scale from 00.1:99.9 to 99.9:0.1, depending upon the specific characteristics desired and the environment in which the material is to function. The nominal formulation which is effective for a typical use is equal amounts of the PTFE with either MoS<sub>2</sub> or WS<sub>2</sub>. For differing applications the mix ratio is skewed to a higher percentage of PTFE within the composite sets when load carrying and wear resistance needs are lower. For higher load and wear resistance requirements the mix ratio is skewed to a higher percentage of MoS<sub>2</sub> or WS<sub>2</sub>, than PTFE. For extreme duty application, i.e., high temperature, high pressure or in a vacuum environment, the composite mix to select is WS<sub>2</sub> with MoS<sub>2</sub>. Such broad load, friction and wear resistance ranges have application in aerospace, pharmaceutical, automotive, paper, packaging, food and virtually any other manufacturing or non-service oriented industry.

In many applications high load pressures are normal, such as with components operating within automotive transmissions, rear axles and engine components under vehicle startup and slow traffic conditions. The effects of wear and friction under these high load and low rpm conditions are the most critical versus when a vehicle attains a steady state condition of fixed velocity highway driving. It is under these high load and low rpm conditions which automotive components are under the highest stress and the effects of friction and wear affect not only component life, but fuel economy as well. Under such conditions this invention will constitute a compound with a higher ratio of MoS<sub>2</sub> or WS<sub>2</sub>, with PTFE. In such an environment, this invention will cause a reduction in frictional horsepower loss which improves fuel economy, engine performance and vehicle drive train component life.

In other applications, generally light load conditions may be normally encountered. Examples of such low pressure range applications include medical equipment, polymer industry applications— injection molding, ejectors pins, etc.; computer components; pharmaceutical products; food, paper and packaging manufacturing and conveying machinery. For such applications this invention will be calibrated to use a higher ratio of PTFE versus high load requirements. This compound will function as a permanent bonded mold release for the polymer industry which will minimize, and in some cases eliminate, the necessity for the millions of cans of aerosol mold release agent used each year. Limiting the use of such aerosol propellants provides a major benefit, not only to the individual exposed these fumes at the press, but also to the long-term effect on the global environment. The use of this invention in medical equipment will allow quieter and cooler running components in equipment such as x-ray, CAT-scan, and external heart pumps. The effects of this invention in this industry would provide longer lasting equipment of better quality and higher production capacity. This will contribute to reduced health care costs.

#### TECHNICAL DISCUSSION

The effectiveness of this invention results from the unique interaction between composite sets of PTFE and MoS<sub>2</sub>, PTFE and WS<sub>2</sub>, or WS<sub>2</sub> and MoS<sub>2</sub>. An integral part of the improved performance of the invention occurs from the dynamic interaction of the lattice layered structure of the MoS<sub>2</sub> and WS<sub>2</sub> and electronegative repulsion occurring in the PTFE molecules. Each constituent of this invention

exists in a similar size sub-micron crystalline structure. This relative uniformity allows a synergistic interaction in the matrix composite between the PTFE and the MoS<sub>2</sub> or WS<sub>2</sub>, as well as between the WS<sub>2</sub> and MoS<sub>2</sub>. When combined in this invention the weak Van der Waals bonding which exists in the MoS<sub>2</sub> and WS<sub>2</sub> molecules, and repulsion of PTFE molecules because of their external electronegativity, increases the composites propensity to shear when pressure is applied. This invention promotes easier shear between its components than the individual constituents experience singularly. In addition, there exists the ability for the composite to work as effectively under higher loads as it will under lighter loads. It further appears that this unique interaction creates a dynamic surface friction and wear-resistant reduction environment beginning at a sub-micron level. The electronegative reaction with the combination of this invention's components appear to create an "additive function", that is the materials combined would tend to have a greater repulsion between themselves than would exist by each singularly. When this invention is applied to a load-carrying surface by any method, such as those presented above, there exists a propensity for the surfaces to repel each other to a greater extent. As a load is applied to this invention, the layer lattice structure of the MoS<sub>2</sub> and the WS<sub>2</sub> constituents yield readily because of the weak bonding between them. The composite sets of PTFE and MoS<sub>2</sub>, or PTFE and WS<sub>2</sub>, interact with the PTFE electronegative charge of the surrounding fluorine atom electrons and gain a slight increase in momentum. This constant interaction occurs on the surface which promotes a dynamic increase in the reduction of friction and improved wear-resistance rather than the normal static form of friction reduction that exists with the PTFE, MoS<sub>2</sub> or WS<sub>2</sub> alone.

Having thus described my invention, it can be seen that various alternative embodiments of the invention can be envisioned without departing from the scope of the invention as defined in the following claims.

I now claim:

1. A particular and specific hybrid series of transition metal polymer matrix composite sets of material consisting of polytetrafluoroethylene and molybdenum disulfide; polytetrafluoroethylene and tungsten disulfide; or tungsten disulfide and molybdenum disulfide.

2. The hybrid series of transition metal polymer matrix composite material sets of claim 1, wherein said mixture includes approximately equal amounts of mixtures of polytetrafluoroethylene with molybdenum disulfide; polytetrafluoroethylene with tungsten disulfide; or, molybdenum disulfide and tungsten disulfide.

3. The hybrid series of transition metal polymer matrix composite material sets of claim 1, wherein said mixture includes a greater amount of molybdenum disulfide with polytetrafluoroethylene, or with tungsten disulfide.

4. The hybrid series of transition metal polymer matrix composite material sets of claim 1, wherein said mixture includes a greater amount of tungsten disulfide with polytetrafluoroethylene, or with molybdenum disulfide.

5. The hybrid series of transition metal polymer matrix composite material sets of claim 1, wherein said mixture includes a greater amount of a polytetrafluoroethylene combined with molybdenum disulfide, or with tungsten disulfide.

6. The hybrid series of transition metal polymer matrix composite material sets of claim 1 wherein said composite material contains at least 75 percent molybdenum disulfide or tungsten disulfide, combined with polytetrafluoroethylene.

7. The hybrid series of transition metal polymer matrix composite material sets of claim 1 wherein said composite material contains at least 75 percent molybdenum disulfide combined with tungsten disulfide.

5 8. The hybrid series of transition metal polymer matrix composite material sets of claim 1 wherein said composite material contains at least 75 percent tungsten disulfide combined with molybdenum disulfide.

9. The hybrid series of transition metal polymer matrix 10 composite material sets of claim 1, wherein said mixture includes at least 75 percent polytetrafluoroethylene combined with molybdenum disulfide, or with tungsten disulfide.

15 10. A method of applying the hybrid series of transition metal polymer composite material sets of claims 1 through 9 to a workpiece wherein said method includes the step of air impingement bonding the powder form of the material to a workpiece using a dry air conveyance.

20 11. A method of applying the hybrid series of transition metal polymer composite material sets of claims 1 through 9 to a workpiece wherein said method including the steps of: providing at least one workpiece; cleaning the surface of said at least one workpiece to remove substantially all contaminants therefrom; and impingement bonding a transition metal polymer matrix composite material sets to at least one workpiece.

25 12. A method as in claim 11, wherein the step of impingement bonding the hybrid series of transition metal polymer matrix composite material sets of claims 1 through 9 onto at least a portion of a workpiece comprises disposing of said composite material in a stream of carrier gas and directing this stream of gas onto at least one workpiece with sufficient force so as to cause said composite material to bond to the surface of said workpiece.

30 13. The method of impingement bonding the hybrid series of transition metal polymer matrix composite material sets as in claim 12, including the further step of pressurizing said gas stream to approximately 30-200 psi.

35 14. A method of applying the hybrid series of transition metal polymer composite material sets of claims 1 through 9 to a substrate, wherein said method includes a mechanical impingement process whereby the workpiece and composite are placed in a rotating container.

40 15. A method of applying the hybrid series of transition metal polymer composite material sets of claims 1 through 9 to a substrate, wherein said method includes the step of a mechanical impingement process whereby the workpiece and composite material are placed in a rotating container which contains an additional compound or associated bur-

50 nishing media.

16. A method of introducing the hybrid series of transition metal polymer composite material sets of claims 1 through 9 to mechanical components by blending the material sets directly in lubricating oils or greases before, or after, said lubricating oils or greases are added to the environment or mechanism desired.

55 17. A method of introducing the hybrid series of transition metal polymer composite material sets of claims 1 through 9 to mechanical components in a liquid environment by converting the material sets, either together or separately, into a colloidal dispersion and introducing this, or these, said solutions into the environment and/or mechanism desired.

60 18. The hybrid series of transition metal polymer composite material sets in colloidal solution of claim 17 premixed with another carrier media, either liquid, dry, semi-solid, or solid, and introducing this solution into the environment and/or mechanism desired.

**19.** The hybrid series of transition metal polymer composite material sets in colloidal solution of claim 17 formed from approximately equal amounts of polytetrafluoroethylene and molybdenum disulfide, equal amounts of polytetrafluoroethylene and tungsten disulfide, or equal amounts of tungsten disulfide and molybdenum disulfide.

**20.** The hybrid series of transition metal polymer composite material sets in colloidal solution of claim 17 formed from a greater amount of polytetrafluoroethylene with molybdenum disulfide, or polytetrafluoroethylene and tungsten disulfide, or, molybdenum disulfide and tungsten disulfide.

**21.** The hybrid series of transition metal polymer composite material sets in colloidal solution of claim 17 formed from at least 75 percent molybdenum disulfide with polytetrafluoroethylene, or 75 percent tungsten disulfide with polytetrafluoroethylene, or 75 percent tungsten disulfide with molybdenum disulfide.

**22.** The hybrid series of transition metal polymer composite material sets in colloidal solution of claim 17 formed from at least 75 percent of polytetrafluoroethylene with molybdenum disulfide, or, 75 percent polytetrafluoroethylene with tungsten disulfide, or, 75 percent molybdenum disulfide with tungsten disulfide.

**23.** The method as in claim 11, wherein the step of impingement bonding the transition metal polymer composite material sets from claims 1 through 9, from a mixture of consisting of approximately equal amounts of either poly-

tetrafluoroethylene and tungsten disulfide, or, polytetrafluoroethylene and molybdenum disulfide, or of tungsten disulfide and molybdenum disulfide.

**24.** The method as in claim 10, wherein the step of impingement bonding the transition metal polymer composite material sets from claims 1 through 9, comprises the step of impingement bonding the composite material consisting of a greater amount of either polytetrafluoroethylene with molybdenum disulfide, or polytetrafluoroethylene and tungsten disulfide, or molybdenum disulfide and tungsten disulfide.

**25.** The method as in claim 10, wherein the step of impingement bonding the transition metal polymer composite material sets from claims 1 through 9, from a mixture of comprises the step of impingement bonding the composite material consisting of at least 75 percent molybdenum disulfide with polytetrafluoroethylene, or 75 percent tungsten disulfide with polytetrafluoroethylene, or 75 percent tungsten disulfide with molybdenum disulfide.

**26.** The method as in claim 10, wherein the step of impingement bonding a material from claims 1 through 9 comprised the step of impingement bonding formed from at least 75 percent of a polytetrafluoroethylene mixed with molybdenum disulfide or, or 75 percent polytetrafluoroethylene with tungsten disulfide, or 75 percent molybdenum disulfide with tungsten disulfide.

\* \* \* \* \*